

# UNITED STATES PATENT OFFICE.

CHARLES BASKERVILLE, OF NEW YORK, N. Y., ASSIGNOR TO THE BASKERVILLE PROCESSES CORPORATION, A CORPORATION OF CONNECTICUT.

## PROCESS OF REFINING SAPONIFIABLE OILS.

1,246,379.

Specification of Letters Patent. Patented Nov. 13, 1917.

No Drawing.

Application filed August 2, 1915. Serial No. 43,297.

*To all whom it may concern:*

Be it known that I, CHARLES BASKERVILLE, a citizen of the United States, residing at New York, in the county of New York and 5 State of New York, have invented certain new and useful Improvements in Processes of Refining Saponifiable Oils, of which the following is a specification.

This invention relates to processes of treating animal and vegetable oils, and more particularly cottonseed oil, for refining and purification, and for decolorizing or bleaching. My complete process preferably utilizes some or all of the processes disclosed in 15 my patents below mentioned, whereby certain combined advantages are secured.

In my prior Patent No. 1,105,743, patented August 4, 1914, I have pointed out that a portion at least of the coloring matter of cotton- 20 seed and similar oils exists in a colloidal state, and is coagulable under the action of certain electrolytes, being thereby rendered easy of removal. In this case the electrolyte is used in presence of an inorganic absorbent 25 having the essential qualities of fuller's earth.

In my prior Patent No. 1,114,095, patented October 20, 1914, I have pointed out that the purification of the oils may be rendered even 30 more satisfactory by the use, in conjunction with fuller's earth, or with fuller's earth and an electrolyte, of an organic absorbent such as suitable forms of cellulose, the action of which is still further enhanced by the addition 35 thereto of an alkali.

The foregoing processes are applicable to the treatment of refined oils. Inasmuch as the filtration processes are facilitated by the presence of the cellulose, it was pointed 40 out in my Patent No. 1,105,744, patented August 4, 1914, that crude oils might be very effectively purified, and the uncombined acid eliminated therefrom, by agitation with cellulose impregnated with alkali, the alkali 45 effectively neutralizing the acid components of the oil with the formation of soaps which were absorbed by the fibrous carrier. In this refining process the usual break is obtained by heating, and the foots, containing 50 the cellulose, are filterable.

In carrying out the above refining process on a large scale, a tendency was observed of the soaps to pass through the filter-cloths and to cloud the oils, involving a subsequent

cleaning with a little fuller's earth. As disclosed, however, in my Patent No. 1,130,698, patented March 9, 1915, this difficulty can be largely obviated by the addition of suitable dehydrating agents, including such anhydrous salts as are capable of taking up water 60 of crystallization, anhydrous sodium carbonate and sulfate being examples. The salts act to harden the soap and thereby reduce its tendency to emulsify with the oil.

My present invention relates to certain improvements in the general process above outlined, whereby the yield of refined oil may be somewhat increased, and valuable products obtained from the foots containing the cellulose.

The cellulose associated with the foots from the filtration persistently retains a material proportion of refined oil, and it has not proven practicable to reduce this proportion materially by any increase in pressure at the 75 filters, when the pressure is exerted by the oil itself, that is to say when the cake is quite wet with oil, containing perhaps as much as 25 per cent. of the whole oil. I have found, however, that an increase of yield of from 80 one to three per cent. of refined oil may be obtained by removing the filter-cakes from the press, and subjecting them, preferably while still warm, to mechanical pressure, for example in a hydraulic or other suitable 85 press. Inasmuch as the additional oil thus obtained is of excellent quality, and no extra costs other than those of pressing are involved, this represents a material economy 90 in the refining process. If, as occurs in some cases, the oil obtained by mechanical pressing carries some soap, it may be added to the next kettle or batch, or it may be cleaned at once, if desired, by the addition 95 of a little fullers' earth followed by filtration under the usual conditions or by washing.

Chemical paper pulp (sulfite pulp) has proven a satisfactory refining agent for use in conjunction with alkali, but entails an 100 extra cost of about fifty cents per ton of oil refined, in addition to the freight to the refinery on the properly prepared pulp. Mechanical paper pulp has not proven satisfactory, because aromatic or tastable substances are extracted from it by the oil under the refining conditions; and moreover, its physical state is not such as to afford the

best results. I have found, however, that "linters" is a very efficient substitute for sulfite pulp, provided it receives suitable preliminary treatment. Ordinary cotton fiber 5 or linters tends to become matted during the stirring, and does not distribute itself properly through the liquid. This difficulty is overcome, however, by cutting it into sufficiently short lengths, about one-fourth inch 10 being suitable, or a very short fibered linters as obtained in some mills may be used without any preliminary treatment. The cut cotton fibers and the short-fiber linters are to be regarded as equivalent for the purposes of 15 this invention. Also, the cotton fibers being tubular, tend to absorb considerable oil; this tendency however can be overcome by wetting them, either with water or with caustic soda solution, just before they are charged 20 into the kettle. The aqueous liquid in the interior of the fiber prevents absorption of oil, and moreover, in case caustic solution is used, the soaps are formed largely in the interior of the fibers from which they do not 25 show the same tendency to escape during filtration and pressing. This wetting, however, is not essential in all cases.

The cake resulting from the process as above described, contains cellulose in the 30 form of linters, soaps and some absorbed oil. By digesting with caustic alkali under usual soap-making conditions, the oil may be saponified, yielding directly a soap product in which a portion of the cellulosic material remains as a filler, some being removed in the process of salting out the soap, and some being actually destroyed during the alkaline digestion for converting the 35 foots into soap.

40 The soap prepared as above is readily converted into soap powder by drying, mixing with a suitable amount of sodium carbonate and pulverizing; and it has been found that in the course of this conversion, the cellulose which it contains is converted in part into a colloidal condition, in which it is quite unobjectionable as a filler, and is not perceptible to the ordinary vision when the soap powder is dissolved in water.

45 50 Or if desired, the pressed cake, instead of being converted into soap, may be "cut" with acid to make the so-called "black grease," which may be drawn off after washing and shipped as such. In the event it is proposed to cut the foots with acid for the manufacture of black grease, it is desirable to use sodium sulfate for the dehydration of the soaps in the refining process; whereas sodium carbonate is to be preferred in case

the cake is to be utilized directly for the 60 manufacture of soap or soap powder.

I claim:—

1. The process of refining saponifiable oils, which consists in treating the oil with linters, separating the bulk of the oil by filtration, and subjecting the resulting cake containing the linters to mechanical pressure to expel a part of the remaining oil. 65

2. The process of refining saponifiable oils and preparing soap products, which consists in treating the oil with an alkali and a cellulosic absorbent, separating the bulk of the oil, and digesting the separated foots, containing the cellulosic absorbent, with alkali for the preparation of a soap product 70 containing a cellulosic filler. 75

3. The process of refining saponifiable oils and preparing soap products, which consists in treating the oil with an alkali and a cellulosic absorbent, separating the bulk of the 80 oil by filtration, subjecting the resulting cake to mechanical pressure to expel a part of the remaining oil, and digesting the pressed foots, containing the cellulosic absorbent, with alkali for the preparation of a soap 85 product containing the cellulosic filler.

4. The process of refining saponifiable oils and preparing soap products, which consists in treating the oil with an alkali and a cellulosic absorbent, separating the bulk of the 90 oil, digesting the separated foots, containing the cellulosic absorbent, with alkali for the preparation of a soap product containing the cellulosic filler, and converting the said soap 95 product into soap powder. 95

5. The process of refining saponifiable oils and preparing soap products, which consists in treating the oil with an alkali and a cellulosic absorbent, separating the bulk of the oil by filtration, subjecting the resulting cake 100 to mechanical pressure to expel a part of the remaining oil, digesting the pressed foots, containing the cellulosic absorbent, with alkali for the preparation of a soap product containing the cellulosic filler, and converting the said soap product into soap powder. 105

6. In a process of refining saponifiable oils, the step which consists in agitating the oil during the refining process with linters impregnated with an aqueous solution of 110 caustic alkali.

In testimony whereof I affix my signature in presence of two witnesses.

CHARLES BASKERVILLE.

Witnesses:

THOMAS F. O'KEEFFE,  
PAUL GROSS.